# EUROPEAN PATENT SPECIFICATION

(11) **EP 0 341 737 B1**
(45) Date of publication and mention of the grant of the patent: **02.01.1992**
(21) Application number: 89108600.1
(22) Date of filing: 12.05.1989
(51) Int. Cl.: C10M 171/00

(54) **Electroviscous fluid**
Elektroviskose Flüssigkeiten
Fluides électro visqueux

(30) Priority: 13.05.1988 JP 116631/88
(43) Date of publication of application: 15.11.1989
(73) Proprietor: MITSUBISHI KASEI CORPORATION, Tokyo 100 (JP)
(72) Inventor: Hattori, Eiji Mitsubishi Kasei Corporation, Yokohama-shi Kanagawa-ken (JP); Oguri, Yasuo Mitsubishi Kasai Corporation, Yokohama-shi Kanagawa-ken (JP)
(74) Representative: Wächtershäuser, Günter, Prof. Dr.

(56) References cited:
- US-A- 3 047 507

## Description

The present invention relates to an electroviscous fluid.

The electroviscous fluid is a fluid showing a so-called electroviscous effect, whereby the apparent viscosity changes quickly and reversibly by the action of applied voltage (off, on, a change in the voltage).

Heretofore, a fluid obtained by vigorously stirring an electrical insulating liquid, fine particles containing or having adsorbed ions and a small amount of water, has been known as one of electroviscous fluids.

The electroviscous effect in such fluid is considered to be brought about as follows.

Namely, by the vigorous stirring, water transfers into fine particles to form an electrolytic solution, and when a voltage is applied, ions in the electrolytic solution are displaced and localized in the fine particles, whereby the particles will be polarized. The respective fine particles flocculate to one another by electrostatic attraction due to the polarization, whereby electroviscous effect will be brought about. There is no particular restriction as to fine particles in such viscous fluid, so long as they are capable of maintaining a dispersed state constantly. Either inorganic or organic fine particles may be employed.

Heretofore, pulverized silica particles have been used as inorganic fine particles, since they are readily available. In a cratch, hydrauric valve, vibration damping device, vibrator or the like wherein the electroviscous fluid is used, it is common to utilize the viscosity change of the fluid when the fluid passes through a space between a pair of electrodes for the application of an electric field. Accordingly, abrasion between the particles as the dispersed phase and the wall of the apparatus creates a problem.

In this respect, the problem of such abrasion is serious with an electroviscous fluid in which pulverized silica particles are employed as the dispersed phase, since the silica particles have sharp edges. An improvement has been desired to solve the problem.

In an electroviscous fluid, particles form a cross-linking structure when a voltage is applied across the electrodes. Accordingly, in the case of pulverized particles, sharp edges of the particles are in contact with one another, whereby there has been a drawback that the dielectric strength tends to be low.

It is an object of the present invention to provide an electroviscous fluid to overcome the above-mentioned problems.

According to the present invention, the object can be readily accomplished by an electroviscous fluid comprising an electrical insulating liquid and fine particles dispersed therein, wherein the fine particles are spherical particles containing an electrolytic solution, obtained by hydrolysis and polycondensation of a metal alkoxide or its derivative.

In the accompanying drawings:
Figure 1 is a scanning electron microscopic photograph showing the structure of spherical silica particles obtained in the Examples given hereinafter.
Figure 2 is a graph showing the viscosity-increasing effect of the electroviscous fluid of Example 1 relative to the applied electric field.

Now, the present invention will be described in detail with reference to the preferred embodiments.

The electroviscous fluid of the present invention employs fine particles dispersed in an insulating liquid, which are spherical particles having an average particle size of from 0.05 to 2 µm obtained by hydrolysis and polycondensation of a metal alkoxide or its derivative. As the metal alkoxide, various alkoxides disclosed in "Metal Alkoxides, edited by D.C. Bradley. R.C. Mehrotra, D.P. Gaur, Academic Press, 1978" may be employed. A preferable alkoxide is composed of lower alkoxy groups of one type or in combination, such as methoxy, ethoxy, propoxy and/or butoxy. Typical examples include alkoxides of e.g. Si, Ti and Zr, and composite alkoxides of e.g. Ba-Ti, Sr-Ti, Pb-Ti, Pb-Ti-Zr and Li-Nb.

The hydrolysis of a metal alkoxide is usually conducted by mixing an alcohol solution of an alkoxide with an aqueous alcohol solution. By properly adjusting the hydrolyzing rate, an amorphous substance of metal oxide can be precipitated substantially in the form of spherical particles. The hydrolyzing rate can usually be adjusted by controlling e.g. the molar ratios and concentrations of the alkoxide and water in the reaction system, and the amount of the catalyst (such as an alkali or acid) for hydrolysis which may be added as the case requires. The conditions to obtain spherical particles can not generally be defined, since they vary depending upon the type of the alkoxide. However, in the case of e.g. Si(OC₂H₅)₄, Ti(OC₂H₅)₄ or Zr(OC₂H₅)₄, the molar ratio of water to the alkoxide is usually from 1 to 150, preferably from 1 to 100, the concentration of the alkoxide is usually from 0.05 to 10 mol/ℓ, preferably from 0.05 dto 5 mol/ℓ, and the concentration of water is usually from 0.1 to 20 mol/ℓ, preferably from 0.1 to 10 mol/ℓ.

Figure 1 shows a scanning electron microscopic photograph (10,000 magnification) of spherical particles of silica obtained by hydrolysis of Si(OC₂H₅)₄ in Example 1. As is evident from the Figure, each particle is spherical, and the particle size distribution is sharp.

Spherical silica particles are obtained by separating the solid content from the alcohol solution by filtration or centrifugal separation, followed by drying by means of e.g. a rotary evaporator and have an average particle size within a range of from 0.05 to 2 µm.

The above spherical particles contain an electrolytic solution, and the electroviscous effect will be obtained by ions in the solution in accordance with the principle as described above.

There is no particular restriction as to the electrolyte constituting the electrolytic solution so long as it dissociates ions in a polar solvent such as water. For example, the electrolyte may be an inorganic compound such as NH₃, NaOH, NaCl, LiCl, B₂O₃, Ca(OH)₂, MgSO₄, Fe(NO₃)₂ or an ionic surfactant such as sodium sulfonate, sodium carboxylate, sodium alkylbenzene sulfonate, sodium polystyrene sulfonate, a calcium salt of fatty acid or a condensation product of naphthalene sulfonic acid with formalin.

Any polar solvent may be used as the solvent constituting the electrolytic solution, so long as it is capable of adequately dissolving the electrolyte used.

The concentration and the content of the electrolytic solution may be suitably selected within the respective ranges not to conduct electricity when the electric field is applied. The concentration is selected usually within a range of from 0.1 to 90% by weight, preferably from 5 to 50% by weight. The content is selected usually within a range of from 0.1 to 20% by weight, preferably from 1 to 10% by weight.

As described above, the hydrolysis and polycondensation of a metal alkoxide can be conducted in the presence a catalyst such as NH₃. In such case, the catalyst can be used by itself as the electrolyte. Namely, after the hydrolysis and polycondensation of a metal alkoxide, spherical silica particles are separated from the alcohol solution and dried. If this drying is not completely conducted but conducted to such an extent that the weight reduction by heating in air upto 200°C would be from 0.1 to 20% by weight, preferably from 1 to 10% by weight, it is possible to obtain spherical particles containing an electrolytic solution within the above-mentioned range. The above-mentioned weight reduction under heating is a value obtained by a differential thermal analysis at a temperature raising rate of 10°C/min.

It is of course possible that the above drying or the preceding washing with water is completely conducted, and an electrolytic solution is subsequently introduced. In such case, it is preferred to use a solvent having a boiling point higher than water, as the polar solvent constituting the electrolytic solution. Namely, with an electroviscous fluid wherein a low boiling solvent such as water is used, there is a problem that when it is used over a long period of time at a high temperature or in an environment where heat is generated by a high shearing force, the solvent will be evaporated or diffused, whereby no adquate electroviscous effect tends to be obtained. By using a solvent having a high boling point, such problem can be solved at once. The polar solvent having a high boling point to be used for this purpose includes glycol (such as ethylene glycol and propylene glycol) and ethanolamine. Among them, ethylene glycol is preferably employed.

To impregnate the particles with the electrolytic solution, the spherical particles, the electrolyte, the polar solvent and the electrical insulating liquid may be mixed for a few hours in e.g. a ball mill, or spherical particles may be impregnated in an electrolyte solution.

As the electrical insulating liquid, a liquid capable of dispersing the spherical particles in a stabilized state, which has a high insulation resistance and which does not dissolve the electrolyte solution, is used. Specifically, it is suitably selected from silicone oil, trans oil, engine oil, an ester, paraffin, an olefin and an aromatic hydrocarbon.

The amount of the spherical particles in the electroviscous fluid is usually from 5 to 50% by volume, perferably from 10 to 40% by volume.

For dispersing, a ball mill or a usual mixing and dispersing machine such as a ultrasonic dispersing machine, may be used.

The electroviscous effect may be measured by using a coaxial double cylinder type rotary viscometer, and an increase in the shearing stress is measured at the same shearing speed (162 sec⁻¹) when a voltage is applied across outer and inner cylinders, and the increase is converted to the change in viscosity.

With the electroviscous fluid, the fluidity can be controlled by the applied voltage. Therefore, its development in the mechatronics field of computer control, is expected. Some examples of the practical application will be mentioned. In the automobile industry, it may be applied to a cratch, a torque converter, a valve, a shock absorber, a brake system or a power steering. Further, in the industrial robot field, it is now being applied to various actuators.

Now, the present invention will be described in further detail with reference to Examples. However, it should be understood that the present invention is by no means restircted to such specific Examples.

### EXAMPLE 1

Solution A obtained by dissolving 186.0 g of Si(OC₂H₅)₄ (guaranteed reagent grade) in 670.7 g of ethyl alcohol (guaranteed reagent grade) and solution B obtained by dissolving 223.6 g of a 28% NH₄OH aqueous solution and 173.9 g of water in 1,999.5 g of ethyl alcohol, were mixed to precipitate silica particles having a diameter of 0.56 µm. The standard deviation from the particle diameter was 1.05. The particles were separated from this slurry by a conventional method and vacuum-dried at 100°C for one hour to obtain particles in a power form. The particles contained NH₃ (1.3 wt%), water (4.1 wt%) and ethanol (0.6 wt%), and the weight reduction was 6% when it was heated in air at 200°C. Then, 30.1 g of the particles were added to 32.8 g of silicone oil (Toray silicone SH200, 10cs), and the mixture was dispersed and mixed for 12 hours in a ball mill.

With respect to the electroviscous fluid of the present invention thus obtained, the shearing stress was measured by using a coaxial double cylinder type rotary viscometer (electrode distance: 1 mm, temperature: 25°C) at the same shearing speed (162 sec⁻¹) when a voltage was applied across the inner and outer cylinders. The results thereby obtained are shown in Figure 2. It is evident that when an electric field 2 kV/mm 1 kV/mm = 10⁶m · kg · S⁻³ · A⁻¹ was applied, the initial viscosity of 1.7 poise increased to a level of 28 poise 1 poise = 10⁻¹ m⁻¹ · kg · S⁻¹. This liquid was left to stand at room temperature, and the measurement was conducted 10 days layer, whereby no change in the properties was observed.

### EXAMPLE 2

Spherical silica particles as used in Example 1 were preliminarily heated at 250°C for 16 hours to adequately remove NH₃, water and ethanol to obtain 40 g of particles. Then, 48 g of a 5.5% NaOH aqueous solution was added thereto, and the mixture was vacuum-dried at 100°C for one hour to obtain particles in a power form. The particles contained NaOH (5.2 wt%) and water (9.7 wt%), and the weight reduction was 9.7% when heated in air at 200°C. Then, 30.1 g of the particles were added to 32.8 g of silicone oil (Toray silicone SH200, 10cs), and the mixture was dispersed and mixed for 12 hours in a ball mill. The initial viscosity of the crude thus obtained was 1.5 poise, and when an electric field of 2 kV/mm was applied, the viscosity increased to 16 poise (162 sec⁻¹).

### EXAMPLE 3

Spherical silica particles as used in Example 1 were preliminarily heated at 250°C for 16 hours to adequately remove NH3, water and ethanol. Then, 10.0 g of silica particles thus obtained and 0.9 g of aqueous ammonia (NH₃ concentration: 25%) were added to 18.7 g of silicone oil (Toray silicone SH200, 10cs), and the mixture was dispersed and mixed for 12 hours in a ball mill. the initial viscosity of the fluid thus obtained was 0.2 poise, and when an electric field of 1.8 kV/mm was applied, the viscosity increased to 22 poise (162 sec⁻¹).

### EXAMPLE 4

Spherical silica particles as used in Example 1 were preliminarily heated at 250°C for 16 hours to adequately remove NH₃, water and ethanol. Then, 10.0 g of the silica particles thus obtained and 1.3 g of an aqueous NaOH solution (NaOH concentration: 44%) were added to 18.7 g of silicone oil (Toray silicone SH200, 10cs), and the mixture was dispersed and mixed for 12 hours in a ball mill. The initial viscosity of the fluid thus obtained was 0.3 poise, and when an electric field of 2 kV/mm was applied, the viscosity increased to 16 poise (162 sec⁻¹).

### EXAMPLE 5

Spherical silica particles as used in Example 1 were preliminarily heated at 250°C for 16 hours to adequately remove NH₃, water and ethanol. Then, 10.0 g of the silica particles thus obtained and 0.7 g of a solution of NaOH in ethylene glycol (NaOH concentration: 1.8%) were added to 18.7 g of silicone oil (Toray silicone SH200, 10cs), and the mixture was dispersed and mixed for 12 hours in a ball mill. The initial viscosity of the fluid thus obtained was 0.8 poise, and when an electric field of 2 kV/mm was applied, the viscosity increased to 17 poise (162 sec⁻¹).

### EXAMPLE 6

20.0 g of spherical silica particles as used in Example 1 were added to 37.1 g of dioctyl adipate (C₈H₁₇OOC(CH₂)₄COOC₈H₁₇), and the mixture was dispersed and mixed for 12 hours in a ball mill. The initial viscosity of the fluid thus obtained was 0.6 poise, and when an electric field of 2 kV/mm was applied, the viscosity increased to 25 poise (162 sec⁻¹).

### EXAMPLE 7

20.0 g of spherial silica particles as used in Example 1 were added to 39.4 g of dioctyl phthalate
and the mixture was dispersed and mixed for 12 hours in a ball mill. The initial viscosity of the fluid thus obtained was 1.1 poise, and when an electric field of 2 kV/mm was applied, the viscosity increased to 37 poise (162 sec⁻¹).

### EXAMPLE 8

20.0 g of spherical silica particles as used in Example 1 were added to a mixture of 7.0 g of a hydrocarbon-type low viscosity mineral oil (Mitsubishi Oil RO-2, 2cs) and 33.4 g of silicone oil (Toray silicone SH200, 5cs), and the mixture was dispersed and mixed for 12 hours in a ball mill. The initial viscosity of the fluid thus obtained was 0.2 poise, and when an electric field of 2 kV/mm was applied, the viscosity increased to 11 poise (162 sec⁻¹).

### COMPARATIVE EXAMPLE 1

Spherical silica particles as used in Example 1 were preliminarily heated at 250°C for 16 hours to adquately remove NH₃, water and ethanol. Then, 10.0 g of the silica particles thus obtained were added to 18.7 g of silicone oil (Toray silicone SH200, 10cs), and the mixture was dispersed and mixed for 12 hours in a ball mill. The electroviscous effect was measured with respect to the fluid thus obtained, whereby no increase in the viscosity was observed.

### COMPARATIVE EXAMPLE 2

Spherical silica particles as used in Example 1 were preliminarily heated at 250°C for 16 hours to adquately remove NH₃, water and ethanol. To 10.0 g of silica particles thus obtained, 10.0 g of distilled water was added, followed by vacuum drying to obtain particles having a water content of 6.8%. Then, 10.0 g of the particles were added to 18.7 g of silicone oil (Toray silicone SH200, 10cs), and the mixture was dispersed and mixed for 12 hours in a ball mill. The electroviscous effect was measured with respect to the fluid thus obtained, whereby no increase in the viscosity was observed.

### COMPARATIVE EXAMPLE 3

Pulverized silica gel was used instead of spherical silica particles in Example 3, and the electroviscous effect was measured, whereby discharge took place when an electric field of 0.5 kV/mm was applied, and subsequent measurement could not be conducted.

As described in the forgoing, the present invention provides an electroviscous fluid having high stability as compared with the compositions disclosed in the prior art.

## Claims

1. An electroviscous fluid comprising an electrical insulating liquid and fine particles dispersed therein, wherein the fine particles are spherical particles containing an electrolytic solution, obtained by hydrolysis and polycondensation of a metal alkoxide or its derivative.

2. The electroviscous fluid according to Claim 1, wherein the electrolytic solution is made of a polar solvent having a higher boiling point than water.

3. The electroviscous fluid according to Claim 2, wherein the polar solvent is ethylene glycol.

4. The electroviscous fluid according to Claim 1, wherein the electrolytic solution has an electrolyte concentration of from 0.1 to 90% by weight, and the electrolytic solution contained in the spherical particles is in an amount of from 0.1 to 20% by weight.

5. The electroviscous fluid according to Claim 1, 2 or 3 wherein the electrolytic solution has an electrolyte concentration of from 5 to 50% by weight, and the electrolytic solution contained in the spherical particles is in an amount of from 1 to 10% by weight.

6. The electroviscous fluid according to Claim 1, wherein the fine particles have an average particle size of from 0.05 to 2 µm.

7. The electroviscous fluid according to Claim 1 or 6, wherein the amount of the fine particles in the electroviscous fluid is from 5 to 50% by volume.

8.The electroviscous fluid according to Claim 1, wherein the metal alkoxide is an alkoxide of at least one member selected from the group consisting of Si, Ti, Zr, Ba-Ti, Sr-Ti, Pb-Ti, Pb-Ti-Zr and Li-Nb.

9. The electroviscous fluid according to Claim 8, wherein the metal alkoxide is composed lower alkoxy groups.

10. The electroviscous fluid according to Claim 8, wherein the metal alkoxide is silicone tetraethoxide.

11. The electroviscous fluid according to Claim 4, wherein the electrolyte is at least one member selected from the group consisting of NH₃, NaOH, NaCl, LiCl, B₂O₃, Ca(OH)₂, MgSO₄, Fe(SO₄)₂, sodium sulfonate, sodium carboxylate, sodium alkylbenzene sulfonate, sodium polystyrene sulfonate, calcium salt of fatty acid and condensation product of naphthalene sulfonic acid with formalin.

## Patentansprüche

1. Elektroviskose Flüssigkeit, umfassend eine elektrisch isolierende Flüssigkeit und darin dispergierte feine Teilchen wobei die feinen Teilchen sphärische Teilchen sind, die eine elektrolytische Lösung enthalten, erhalten durch Hydrolyse und Polykondensation eines Metallalkoxids oder dessen Derivat.

2. Elektroviskose Flüssigkeit gemäß Anspruch 1, wobei die elektrolytische Lösung aus einem polaren Lösungsmittel mit einem höheren Siedepunkt als Wasser hergestellt wurde.

3. Elektroviskose Flüssigkeit gemäß Anspruch 2, wobei das polare Lösungsmittel Ethylenglycol ist.

4. Elektroviskose Flüssigkeit gemäß Anspruch 1, wobei die elektrolytische Lösung eine Elektrolytkonzentration von 0,1 bis 90 Gew.-% aufweist und die in den sphärischen Teilchen enthaltene elektrolytische Lösung in einer Menge von 0,1 bis 20 Gew.-% vorliegt.

5. Elektroviskose Flüssigkeit gemäß Anspruch 1, 2 oder 3, wobei die elektrolytische Lösung eine Elektrolytkonzentration von 5 bis 50 Gew.-% aufweist und die in den sphärischen Teilchen enthaltene elektrolytische Lösung in einer Menge von 1 bis 10 Gew.-% vorliegt.

6. Elektroviskose Flüssigkeit gemäß Anspruch 1, wobei die feinen Teilchen eine durchschnittliche Teilchengröße von 0,05 bis 2 µm aufweisen.

7. Elektroviskose Flüssigkeit gemäß Anspruch 1 bis 6, wobei die Menge der feinen Teilchen in der elektroviskosen Flüssigkeit von 5 bis 50 Vol.-% ausmacht.

8. Elektroviskose Flüssigkeit gemäß Anspruch 1, wobei das Metallalkoxid ein Alkoxid von mindestens einem Mitglied, ausgewählt aus der Gruppe bestehend aus Si, Ti, Zr, Ba-Ti, Sr-Ti, Pb-Ti, Pb-Ti-Zr und Li-Nb, ist.

9. Elektroviskose Flüssigkeit gemäß Anspruch 8, wobei das Metallalkoxid Niederalkoxygruppen aufweist.

10. Elektroviskose Flüssigkeit gemäß Anspruch 8, wobei das Metallalkoxid Siliciumtetraethoxid ist.

11. Elektroviskose Flüssigkeit gemäß Anspruch 4, wobei der Elektrolyt mindestens ein Mitglied, ausgewählt aus der Gruppe bestehend aus NH₃, NaOH, NaCl, LiCl, B₂O₃, Ca(OH)₂, MgSO₄, Fe(SO₄)₂, Natriumsulfonat, Natriumcarboxylat, Natriumalkylbenzolsulfonat, Natriumpolystyrolsulfonat, Calciumsalz von Fettsäure und Kondensationsprodukt von Naphthalinsulfonsäure mit Formalin, ist.

## Revendications

1. Fluide électrovisqueux comprenant un liquide d'isolation électrique et de fines particules dispersées en son sein, dans lequel les fines particules sont des particules sphériques contenant une solution électrolytique, obtenues par hydrolyse et polycondensation d'un alcoolate métallique ou de son dérivé.

2. Fluide électrovisqueux selon la revendication 1, dans lequel la solution électrolytique est faite d'un solvant polaire ayant un point d'ébullition supérieur à celui de l'eau.

3. Fluide électrovisqueux selon la revendication 2, dans lequel le solvant polaire est l'éthylène glycol.

4. Fluide électrovisqueux selon la revendication 1, dans lequel la solution électrolytique a une concentration en électrolyte de 0,1 à 90% en poids, et la solution électrolytique contenue dans les particules sphériques est présente dans une quantité de 0,1 à 20% en poids.

5. Fluide électrovisqueux selon la revendication 1, 2 ou 3, dans lequel la solution électrolytique a une concentration en électrolyte de 5 à 50% en poids, et la solution électrolytique contenue dans les particules sphériques est présente dans une quantité de 1 à 10% en poids.

6. Fluide électrovisqueux selon la revendication 1, dans lequel les fines particules ont une dimension moyenne de particule de 0,05 à 2 µm.

7. Fluide électrovisqueux selon la revendication 1 ou 6, dans lequel la quantité des fines particules présentes dans le fluide électrovisqueux est de 5 à 50% en volume.

8. Fluide électrovisqueux selon la revendication 1, dans lequel l'alcoolate métallique est un alcoolate d'au moins un élément choisi dans le groupe constitué par Si, Ti, Zr, Ba-Ti, Sr-Ti, Pb-Ti, Pb-Ti-Zr et Li-Nb.

9. Fluide électrovisqueux selon la revendication 8, dans lequel l'alcoolate métallique est composé de groupes alcoxy inférieurs.

10. Fluide électrovisqueux selon la revendication 8, dans lequel l'alcoolate métallique est le tétraéthylate de silicium.

11. Fluide électrovisqueux selon la revendication 4, dans lequel l'électrolyte est au moins un élément choisi dans le groupe constitué par NH₃, NaOH, NaCl, LiCl, B₂O₃, Ca(OH)₂, MgSO₄, Fe(SO₄)₂, le sulfonate de sodium, le carboxylate de sodium, l'alkylbenzène sulfonate de sodium, le polystyrène sulfonate de sodium, les sels de calcium d'acides gras et les produits de condensation de l'acide naphtalène sulfonique avec le formol.
